

## PHOTOGRAPHIC EMULSIONS

Thomas David Smith, Red Bank, N.J., assignor to E. I. du Pont de Nemours and Company, Wilmington, Del., a corporation of Delaware

No Drawing. Filed May 1, 1957, Ser. No. 656,195

11 Claims. (Cl. 96—107)

This invention relates to photographic silver halide emulsions containing a non-optical sensitizing agent having at least one polyoxyalkylene group. More particularly it relates to such emulsions containing a hydrocarbon-substituted mononuclear monohydric phenol of at least 10 carbon atoms wherein a hydrocarbon substituent is in the para-position to the hydroxyl group. The invention also relates to photographic elements bearing at least one layer of such an emulsion.

It is known that photographic silver halide emulsions which have been sensitized to very high levels tend to produce fog on development. This photographic fog is due to the existence in the emulsion of silver halide grains which are developable without exposure to light. In addition, fog may be produced in photographic emulsions during storage, particularly under adverse conditions of temperature and humidity.

As is well known, the sensitivity of photographic emulsions can be increased in a number of ways. One of these is by adding derivatives of alkylene oxides, such as polyalkylene oxides or condensation products of alkylene oxides or polyalkylene oxides, e.g., ethylene oxide, with acids, alcohols or amines as disclosed in U.S. patents Blake et al. 2,400,532, Blake 2,423,549, Blake 2,441,389 and Carroll et al. 2,716,062. However, these compounds tend to cause fog when photographic materials, the emulsions of which contain them, are stored for any length of time. Attempts to reduce this fog have involved the use of antifogging agents which are frequently detrimental to certain photographic properties. In particular, certain such agents tend to reduce the photographic speed of film when exposed to relatively low intensity illumination.

It is therefore an object of this invention to provide means for reducing fog in photographic emulsions. Another object is to reduce fog produced on storage of emulsions, particularly in tropical climates or under other adverse conditions of temperature and humidity. A further object of this invention is to provide silver halide emulsions sensitized with alkylene oxide polymers and of improved stability and less tendency to form an objectionable amount of fog on normal storage and photographic elements embodying such emulsions. Still other objects are to achieve the above results without reducing speed or contrast and, in particular, without reducing the speed of the emulsion to low intensity illumination.

The above objects are attained in accordance with the invention, and photographic emulsions of good stability, speed and contrast and exhibiting low fog values upon aging at normal temperatures or for extended periods of time are provided by admixing relatively small amounts of at least one hydrocarbon-substituted mononuclear monohydric phenol of at least 9 carbon atoms with a photographic silver halide emulsion containing sensitizing amounts of a non-optical or chemical emulsion sensitizing agent having a molecular weight of at least 282 and containing at least two and preferably at least six oxyalkylene units of 2 to 4 carbon atoms.

The mononuclear monohydric phenols used in accord-

ance with the invention, in addition to the hydrocarbon substituent in the para-position to the hydroxyl group, may contain one, two or three additional hydrocarbon substituents in the benzene ring containing the phenolic hydroxyl group. Among the hydrocarbon substituents which may be present in the para-position and in the other positions of the benzene ring are alkyl radicals of 1 to 18 carbon atoms, e.g., methyl, ethyl, n-propyl, isopropyl, t-butyl, sec-amyl, t-amyl, t-octyl, n-nonyl and n-dodecyl; aryl, e.g., phenyl, naphthyl and bi-phenyl; aralkyl, e.g., benzyl,  $\alpha$ -cumyl and naphthylmethyl, and cycloalkyl, e.g., cyclopentyl and cyclohexyl. In an important specific embodiment of the invention, the hydrocarbon substituted mononuclear monohydric phenols have at least one t-butyl substituent in the molecule.

It has been found that when 5 to 50 millimoles of a hydrocarbon-substituted mononuclear monohydric phenol described above is added per mole of silver halide to the sensitized emulsions that the speed (i.e., response of the emulsion to radiation of both high and low intensity), contrast and fog values of the resulting emulsions remain substantially at the initial values of the emulsion, even when the emulsions or emulsion layers are maintained under adverse storage conditions for short or extended periods of time, e.g., at an elevated temperature and/or high conditions of humidity.

The invention is not limited to any particular type of light-sensitive silver halide as it is useful with silver chloride, silver bromide, silver iodobromide, silver chlorobromide, etc., emulsions and mixed emulsions of these types. It is particularly efficacious in silver iodobromide emulsions containing about 2 mole percent iodide and the rest bromide. These emulsions may be sensitized by means of non-optical or chemical sensitizing agents other than the polyoxyalkylene polymers mentioned above. Thus, noble metal sensitizers, e.g., gold compounds, e.g., chlorauric acid and auric trichloride, may be present in association with sulfur sensitizers containing labile sulfur, e.g., sodium thiosulfate, allylthiocarbamide, alkali metal thiocyanates, sodium sulfide, and allylthiourea. These sensitizers are generally used in amounts of 0.005% or less based on the weight of the silver halide. Moreover, the silver halide emulsions may contain one or more optical sensitizing agents, e.g., cyanine, carbocyanine, merocyanine pseudocyanine, cyazine, etc., dyes.

With regard to the non-optical sensitizers which contain at least one polyoxyalkylene group, there are a relatively large number of such compounds known to the art, suitable compounds being described in the above-identified patents. These compounds include not only the polyalkylene oxides or glycols wherein the oxyalkylene groups contain 2 to 4 carbon atoms but also the condensation products of alkylene oxides of 2 to 4 carbon atoms with glycols, fatty acids, saturated aliphatic amines, and hexitol ring dehydration products, said compounds having a molecular weight of at least 282, suitable specific compounds of which are disclosed in the aforesaid patents. In general these sensitizing compounds are present in amounts from 0.1 to 2.0 g. per mole of silver halide. While gelatin is the preferred binding agent for the silver halide grains, other water-permeable amphoteric protein protective colloids, e.g., albumin and casein, can be used. Also, agar-agar, alginic acid and the alginates, polyglycuronic acid, polyvinyl alcohol, polyvinyl acetals including those containing color forming nuclei, and other natural or synthetic water permeable colloids useful in making photographic emulsions can be used as the original colloid during the precipitation, or in the final emulsion as bulk ing agents.

The hydrocarbon-substituted mononuclear monohydric phenols are preferably added to the silver halide emulsion after it has been brought to its maximum sensitivity.

and the conventional adjuvants are added just prior to coating onto a suitable support to form a photographic element. They can, of course, be added at an earlier stage, that is, at the time of second digestion.

The invention will now be further illustrated by, but is not intended to be limited to, the following examples wherein the silver halide weight ratio, unless otherwise indicated, is 1.6 mole percent iodide and the remainder bromide.

## Example 1

10

A high speed gelatino-silver iodobromide emulsion was digested with an organic sulfur compound and gold chloride. After digestion the emulsion was divided into three portions. One portion was treated with 0.5 gram of a condensation product of polyethylene oxide with oleyl alcohol having a molecular weight of approximately 900 ("Emulphor" ON-870 manufactured by the Antara Chemicals Division, General Aniline and Film Corp.) per mole of silver halide. To a second portion was added 0.5 gram of said condensation product together with 20 millimoles of 2-benzyl-4-methyl-6-t-butylphenol, which is disclosed and claimed in assignee's Pickl and Stevenson U.S. application Ser. No. 494,262 filed Mar. 14, 1955, per mole of silver halide. A third portion having neither of these additions was used as a control. The emulsions were coated on cellulose acetate film base and were exposed to X-rays in the presence of an intensifying screen at two different intensity levels. The exposure of greater intensity has been designated as No. 2 and that of lower intensity and longer time as No. 1.

The coatings were developed for 5 minutes in a developer of the following composition:

|                               | grams | 35  |
|-------------------------------|-------|-----|
| Metol                         |       | 3   |
| Anhydrous sodium sulfite      |       | 50  |
| Hydroquinone                  |       | 9   |
| Anhydrous potassium carbonate |       | 50  |
| Potassium bromide             |       | 4.5 |
| Water to make 1000 ml.        |       | 40  |

The coatings were tested fresh, after two months of room aging, and after one week at 120° F. and 65% R.H. (relative humidity). The aged materials were exposed and developed as described above. Results of tests for speed, gamma and fog, before and after the storage treatment of each of the samples, are given below. Speed is given in terms of a reciprocal of exposure at a density of 0.7. If fog is greater than 0.40 the speed and gamma numbers are of no significance and are therefore not included in such cases.

## FRESH RESULTS

| Compound                                  | Amount per Mole          | No. 2 Exposure |       | No. 1 Exposure |       | Fog |
|-------------------------------------------|--------------------------|----------------|-------|----------------|-------|-----|
|                                           |                          | Speed          | Gamma | Speed          | Gamma |     |
| Control                                   | None                     | 940            | 2.67  | 450            | 2.43  | .15 |
| Polyoxyethylated oleyl alcohol (I).       | 0.5 g.                   | 1,040          | 3.02  | 520            | 2.52  | .30 |
| I plus 2-benzyl-4-methyl-6-t-butylphenol. | 0.5 g.<br>20 millimoles. | 1,010          | 2.43  | 510            | 2.49  | .16 |

## 2 MONTHS ROOM AGING

| Compound                 | No. 2 Exposure |       | No. 1 Exposure |       | Fog |
|--------------------------|----------------|-------|----------------|-------|-----|
|                          | Speed          | Gamma | Speed          | Gamma |     |
| Control                  | 640            | 2.45  | 320            | 2.00  | .23 |
| I                        |                |       |                |       |     |
| I plus phenolic compound | 670            | 2.45  | 340            | 1.97  | .22 |

75

ONE WEEK AT 120° F. AND 65% R.H.

| Compound                 | Fog |
|--------------------------|-----|
| Control                  | .24 |
| I plus phenolic compound | .78 |

## Example 2

A gelatino-silver iodobromide emulsion, digested with sulfur and gold compounds, was divided into three portions. One portion was treated with .67 g. of polyethylene oxide monostearate having an average molecular weight of from 950-1050 ("Carbowax" 1000 monostearate manufactured by the Glyco Products Company) per mole of silver halide. To a second portion there was added .67 g. of the polyethylene oxide monostearate per mole of silver halide together with 5.0 millimoles of 2-benzyl-4-methyl-6-t-butylphenol (II) per mole of silver halide. Neither of these additions were made to a third portion, which was used as a control.

Coating, exposure and development were carried out as in Example 1. Aging tests for 2 months under normal room conditions were carried out with the following results.

## FRESH RESULTS

| Compound                          | Amount per Mole       | No. 2 Exposure |       | No. 1 Exposure |       | Fog |
|-----------------------------------|-----------------------|----------------|-------|----------------|-------|-----|
|                                   |                       | Speed          | Gamma | Speed          | Gamma |     |
| Control                           | None                  | 850            | 2.22  | 420            | 2.13  | .13 |
| I Polyethylene oxide monostearate | .67                   | 1,000          | 2.46  | 440            | 2.22  | .16 |
| I plus II                         | .67<br>5.0 millimoles | 960            | 2.68  | 440            | 2.55  | .14 |

## 2 MONTHS ROOM AGING

| Compound  | No. 2 Exposure |       | No. 1 Exposure |       | Fog |
|-----------|----------------|-------|----------------|-------|-----|
|           | Speed          | Gamma | Speed          | Gamma |     |
| Control   | 630            | 2.03  | 320            | 1.76  | .20 |
| I         | 700            | 2.31  | 330            | 1.76  | .28 |
| I plus II | 740            | 2.32  | 380            | 1.95  | .22 |

## Example 3

A gelatino-silver iodobromide emulsion, digested with sulfur and gold compounds, was divided into three portions. One portion was treated with .67 gram of a polyethylene oxide having an average molecular weight of 6000-7500 ("Carbowax 6000") per mole of silver halide. To a second portion were added .67 gram of the polyethylene oxide together with 16.7 millimoles of 2-benzyl-4-methyl-6-t-butylphenol (II) per mole of silver halide. Neither of these additions was made to a third portion of the emulsion.

Coating, exposure, development and aging were carried out as in Example 1.

## FRESH RESULTS

| Compound               | Amount per Mole | No. 2 Exposure |       | No. 1 Exposure |       | Fog |
|------------------------|-----------------|----------------|-------|----------------|-------|-----|
|                        |                 | Speed          | Gamma | Speed          | Gamma |     |
| Control                | None            | 950            | 3.11  | 460            | 2.72  | .18 |
| Polyethylene oxide (I) | .67             | 1,170          | 3.08  | 530            | 2.70  | .24 |
| I plus II              | .67<br>16.7     | 1,070          | 3.10  | 520            | 2.89  | .22 |

## 2 MONTHS ROOM AGING

| Compound       | No. 2 Exposure |       | No. 1 Exposure |       | Fog  |
|----------------|----------------|-------|----------------|-------|------|
|                | Speed          | Gamma | Speed          | Gamma |      |
| Control.....   | 660            | 2.39  | 390            | 2.15  | .21  |
| I.....         |                |       |                |       | 2.01 |
| I plus II..... | 960            | 3.00  | 460            | 2.34  | .25  |

ONE WEEK AT 120° F. AND 65% R.H.

| Compound       | Fog  |
|----------------|------|
| Control.....   | .40  |
| I.....         | 3.20 |
| I plus II..... | .48  |

The "Carbowax 6000" referred to above is manufactured by the Carbide and Carbon Chemicals Company.

## Example 4

A gelatino-silver iodobromide emulsion, digested with sulfur and gold compounds, was divided into three portions. One portion was treated with .53 g. of the polyethylene oxide described in Example 3 per mole of silver halide. To a second portion were added .53 g. of the polyethylene oxide and 20 millimoles 2,3,6-t-butyl-4-phenylphenol (II) per mole of silver halide. The preparation of this phenol will be found in J. Chem. Ed. 32, 312 (1955). Neither of these additions was made to a third portion of the emulsion.

Coating, exposure, development and aging were carried out as in Example 1 except that the emulsions were tested after one month of room temperature aging.

## FRESH RESULTS

| Compound                  | Amount per Mole    | No. 2 Exposure |       | No. 1 Exposure |       | Fog |
|---------------------------|--------------------|----------------|-------|----------------|-------|-----|
|                           |                    | Speed          | Gamma | Speed          | Gamma |     |
| Control.....              | None.....          | 850            | 2.49  | 350            | 2.13  | .23 |
| I Polyethylene oxide..... | .53 g.....         | 1,240          | 2.35  | -----          | ----- | .46 |
| I plus.....               | .53 g.....         | 820            | 2.60  | 540            | 2.12  | .14 |
| II.....                   | 20 millimoles..... |                |       |                |       |     |

ONE MONTH ROOM AGING

| Compound       | No. 2 Exposure |       | No. 1 Exposure |       | Fog  |
|----------------|----------------|-------|----------------|-------|------|
|                | Speed          | Gamma | Speed          | Gamma |      |
| Control.....   |                |       |                |       | 1.46 |
| I plus II..... | 640            | 2.41  | 340            | 1.89  | .22  |

ONE WEEK AT 120° F. AND 65% R.H.

| Compound       | Fog  |
|----------------|------|
| Control.....   | .24  |
| I.....         | 2.51 |
| I plus II..... | .24  |

## Example 5

A gelatino-silver bromoiodide emulsion, digested with sulfur and gold compounds, was divided into three portions. One portion was treated with .53 g. of the polyethylene oxide described in Example 3 ("Carbowax 6000") per mole of silver halide. To a second portion was added .53 g. of the polyethylene oxide and 20 millimoles p-n-nonylphenol (II) per mole of silver halide. Neither of these additions were made to a third portion of the emulsion.

Coating, exposure, development and aging were carried out as in Example 4.

## FRESH RESULTS

| Compound                    | Amount per Mole    | No. 2 Exposure |       | No. 1 Exposure |       | Fog |
|-----------------------------|--------------------|----------------|-------|----------------|-------|-----|
|                             |                    | Speed          | Gamma | Speed          | Gamma |     |
| Control.....                | None.....          | 720            | 2.38  | 390            | 2.04  | .20 |
| Polyethylene oxide (I)..... | .53 g.....         | -----          | ----- | -----          | ----- | .55 |
| I plus.....                 | .53 g.....         | 720            | 2.77  | 390            | 2.48  | .23 |
| II.....                     | 20 millimoles..... |                |       |                |       |     |

ONE MONTH ROOM AGING

| Compound       | No. 2 Exposure |       | No. 1 Exposure |       | Fog |
|----------------|----------------|-------|----------------|-------|-----|
|                | Speed          | Gamma | Speed          | Gamma |     |
| Control.....   | 640            | 1.92  | 330            | 1.52  | .17 |
| I.....         | 680            | 2.46  | 390            | 2.17  | .22 |
| I plus II..... |                |       |                |       |     |

ONE WEEK AT 120° F. AND 65% R.H.

| Compound       | Fog  |
|----------------|------|
| Control.....   | .26  |
| I.....         | 1.95 |
| I plus II..... | .28  |

## Example 6

30 A gelatino-silver iodobromide emulsion, digested with sulfur and gold compounds, was divided into three portions. One portion was treated with .53 g. of a polyethylene oxide described in Example 3 ("Carbowax 6000") per mole of silver halide. To a second portion was added .53 g. of the polyethylene oxide together with 20 millimoles 2,4 di-n-nonylphenol (II) per mole of silver halide. Neither of these additions was made to a third portion of the emulsion.

Coating, exposure, development and aging were carried out as in Example 4.

## FRESH RESULTS

| Compound                    | Amount per Mole    | No. 2 Exposure |       | No. 1 Exposure |       | Fog |
|-----------------------------|--------------------|----------------|-------|----------------|-------|-----|
|                             |                    | Speed          | Gamma | Speed          | Gamma |     |
| Control.....                | None.....          | 720            | 2.38  | 390            | 2.04  | .20 |
| Polyethylene oxide (I)..... | .53 g.....         | -----          | ----- | -----          | ----- | .55 |
| I plus.....                 | .53 g.....         | 690            | 2.88  | 400            | 2.71  | .21 |
| II.....                     | 20 millimoles..... |                |       |                |       |     |

ONE MONTH ROOM AGING

| Compound       | No. 2 Exposure |       | No. 1 Exposure |       | Fog |
|----------------|----------------|-------|----------------|-------|-----|
|                | Speed          | Gamma | Speed          | Gamma |     |
| Control.....   | 640            | 1.92  | 330            | 1.52  | .17 |
| I.....         | 720            | 2.43  | 370            | 1.95  | .20 |
| I plus II..... |                |       |                |       |     |

ONE WEEK AT 120° F. AND 65% R.H.

| Compound       | Fog  |
|----------------|------|
| Control.....   | .26  |
| I.....         | 1.95 |
| I plus II..... | .85  |

## Example 7

70 A gelatino-silver iodobromide emulsion, digested with sulfur and gold compounds, was divided into three portions. One portion was treated with .53 g. of the polyethylene oxide described in Example 3 ("Carbowax") per

mole of silver halide. To a second portion was added .53 g. of the polyethylene oxide together with 20 millimoles p-n-dodecylphenol (II) per mole of silver halide. Neither of these additions was made to a third portion of the emulsion.

Coating, exposure, development and aging were carried out as in Example 4.

## FRESH RESULTS

| Compound                         | Amount per Mole          | No. 2 Exposure |       | No. 1 Exposure |       | Fog  |  |
|----------------------------------|--------------------------|----------------|-------|----------------|-------|------|--|
|                                  |                          | Speed          | Gamma | Speed          | Gamma |      |  |
|                                  |                          |                |       |                |       |      |  |
| Control                          |                          | 720            | 2.38  | 390            | 2.04  | .20  |  |
| Polyethylene oxide (I).          | .53 g.                   |                |       |                |       | .55  |  |
| I plus II                        | .53 g.<br>20 millimoles. | 730            | 3.16  | 390            | 2.49  | .23  |  |
| ONE MONTH ROOM AGING             |                          |                |       |                |       |      |  |
| Compound                         | Amount per Mole          | No. 2 Exposure |       | No. 1 Exposure |       | Fog  |  |
|                                  |                          | Speed          | Gamma | Speed          | Gamma |      |  |
|                                  |                          |                |       |                |       |      |  |
| Control                          |                          | 640            | 1.92  | 330            | 1.52  | .17  |  |
| I                                |                          |                |       |                |       | .76  |  |
| I plus II                        |                          | 670            | 2.51  | 330            | 2.37  | .20  |  |
| ONE WEEK AT 120° F. AND 65% R.H. |                          |                |       |                |       |      |  |
| Compound                         | Amount per Mole          | No. 2 Exposure |       | No. 1 Exposure |       | Fog  |  |
|                                  |                          | Speed          | Gamma | Speed          | Gamma |      |  |
|                                  |                          |                |       |                |       |      |  |
| Control                          |                          |                |       |                |       | .26  |  |
| I                                |                          |                |       |                |       | 1.95 |  |
| I plus II                        |                          |                |       |                |       | .31  |  |

## Example 8

A gelatino-silver iodobromide emulsion, digested with sulfur and gold compounds, was divided into three portions. One portion was treated with .53 g. of the condensation product of Example 1 ("Emulphor" ON-870) per mole of silver halide. To a second portion was added .53 g. of the above condensation product together with 5 millimoles of t-octylphenol



per mole of silver halide. Neither of these additions was made to a third portion of the emulsion which served as a control.

Coating, exposure, development and aging were carried out as in Example 1 and the fresh results and one week at 120° F. and 65% R.H. are as follows:

## FRESH RESULTS

| Compound                            | Amount per Mole         | No. 2 Exposure |       | No. 1 Exposure |       | Fog |  |
|-------------------------------------|-------------------------|----------------|-------|----------------|-------|-----|--|
|                                     |                         | Speed          | Gamma | Speed          | Gamma |     |  |
|                                     |                         |                |       |                |       |     |  |
| Control                             | None                    | 980            | 2.89  |                |       |     |  |
| Polyoxyethylated oleyl alcohol (I). | .53                     | 1,140          | 3.02  | 460            | 2.46  | .24 |  |
| I plus II                           | .53 g.<br>5 millimoles. | 1,060          | 3.34  | 440            | 2.61  | .20 |  |
| ONE WEEK AT 120° F. AND 65% R.H.    |                         |                |       |                |       |     |  |
| Compound                            | Amount per Mole         | No. 2 Exposure |       | No. 1 Exposure |       | Fog |  |
|                                     |                         | Speed          | Gamma | Speed          | Gamma |     |  |
|                                     |                         |                |       |                |       |     |  |
| Control                             |                         |                |       |                |       | .24 |  |
| I                                   |                         |                |       |                |       | .34 |  |
| I plus II                           |                         |                |       |                |       | .21 |  |

75  
ONE WEEK AT 120° F. AND 65% R.H.  
Compound  
Fog  
Control  
I  
I plus II  
70  
Compound  
Fog  
Control  
I  
I plus II  
75

8  
Example 9

A gelatino-silver iodobromide emulsion, digested with sulfur and gold compounds, was divided into three portions. One portion was treated with .27 g. of the polyethylene oxide described in Example 3 ("Carbowax 6000") per mole of silver halide. To a second portion was added 0.27 g. of the polyethylene oxide and a mixture (II) of 8 millimoles of 2-benzyl-4-methyl-6-t-butylphenol and 2 millimoles of 2,3,6-tri-t-butyl-4-phenylphenol per mole of silver halide.

Coating, exposure, development and aging were carried out as in Example 4.

## FRESH RESULTS

| Compound                | Amount per Mole          | No. 2 Exposure |       | No. 1 Exposure |       | Fog |  |
|-------------------------|--------------------------|----------------|-------|----------------|-------|-----|--|
|                         |                          | Speed          | Gamma | Speed          | Gamma |     |  |
|                         |                          |                |       |                |       |     |  |
| Control                 | None                     | 1,030          | 2.70  | 420            | 2.48  | .28 |  |
| Polyethylene oxide (I). | .27 g.                   | 1,080          | 3.08  | 480            | 2.48  | .32 |  |
| I plus II               | .27 g.<br>10 millimoles. | 1,048          | 3.06  | 460            | 2.47  | .18 |  |
| ONE MONTH ROOM AGING    |                          |                |       |                |       |     |  |

## ONE MONTH ROOM AGING

| Compound                         | Amount per Mole | No. 2 Exposure |       | No. 1 Exposure |       | Fog |  |
|----------------------------------|-----------------|----------------|-------|----------------|-------|-----|--|
|                                  |                 | Speed          | Gamma | Speed          | Gamma |     |  |
|                                  |                 |                |       |                |       |     |  |
| Control                          |                 | 840            | 2.53  | 370            | 1.99  | .32 |  |
| I                                |                 |                |       |                |       | .70 |  |
| I plus II                        |                 | 880            | 2.73  | 400            | 2.21  | .38 |  |
| ONE WEEK AT 120° F. AND 65% R.H. |                 |                |       |                |       |     |  |

| Compound  | Amount per Mole | No. 2 Exposure |       | No. 1 Exposure |       | Fog  |  |
|-----------|-----------------|----------------|-------|----------------|-------|------|--|
|           |                 | Speed          | Gamma | Speed          | Gamma |      |  |
|           |                 |                |       |                |       |      |  |
| Control   |                 |                |       |                |       | .56  |  |
| I         |                 |                |       |                |       | 2.12 |  |
| I plus II |                 |                |       |                |       | 0.38 |  |

## Example 10

A gelatino-silver iodobromide emulsion, digested with sulfur and gold compounds, was divided into three portions. One portion was treated with 1.1 g. polyoxyethylated oleyl alcohol of Example 1 per mole of silver halide. To a second portion was added 1.1 g. of the above condensation product per mole of silver halide together with 20 millimoles of p-t-butylphenol (II).

Coating, exposure, development and aging were carried out as in Example 1.

## FRESH RESULTS

| Compound                            | Amount per Mole          | No. 2 Exposure |       | No. 1 Exposure |       | Fog |  |
|-------------------------------------|--------------------------|----------------|-------|----------------|-------|-----|--|
|                                     |                          | Speed          | Gamma | Speed          | Gamma |     |  |
|                                     |                          |                |       |                |       |     |  |
| Control                             | None                     | 720            | 2.27  | 440            | 2.01  | .38 |  |
| Polyoxyethylated oleyl alcohol (I). | 1.1 g.                   |                |       |                |       | .82 |  |
| I plus II                           | 1.1 g.<br>20 millimoles. | 880            | 2.63  | 450            | 2.19  | .40 |  |
| ONE MONTH ROOM AGING                |                          |                |       |                |       |     |  |

| Compound  | Amount per Mole | No. 2 Exposure |       | No. 1 Exposure |       | Fog |  |
|-----------|-----------------|----------------|-------|----------------|-------|-----|--|
|           |                 | Speed          | Gamma | Speed          | Gamma |     |  |
|           |                 |                |       |                |       |     |  |
| Control   |                 |                |       |                |       | .56 |  |
| I         |                 |                |       |                |       | .74 |  |
| I plus II |                 | 750            | 2.47  | 470            | 2.19  | .38 |  |

ONE WEEK AT 120° F. AND 65% R.H.

| Compound  |  | Fog  |
|-----------|--|------|
| Control   |  | .48  |
| I         |  | 1.60 |
| I plus II |  | .66  |

## Example 11

A gelatino-silver iodobromide emulsion, digested with sulfur and gold compounds, was divided into three portions. One portion was treated with .5 g. of the polyoxyethylated oleyl alcohol of Example 1 per mole of silver halide. To a second portion was added .5 g. of the above condensation product per mole of silver halide together with 20 millimoles of p-benzylphenol (II).

Coating, exposure, development and aging were carried out as in Example 4.

## FRESH RESULTS

| Compound                            | Amount per Mole         | No. 2 Exposure |       | No. 1 Exposure |       | Fog |
|-------------------------------------|-------------------------|----------------|-------|----------------|-------|-----|
|                                     |                         | Speed          | Gamma | Speed          | Gamma |     |
| Control                             | None                    | 720            | 2.27  | 320            | 2.01  | .38 |
| Polyoxyethylated oleyl alcohol (I). | .5 g.                   |                |       |                |       | .72 |
| I plus II                           | .5 g.<br>20 millimoles. | 840            | 2.49  | 340            | 2.15  | .26 |

## ONE MONTH ROOM AGING

| Compound  | Amount per Mole | No. 2 Exposure |       | No. 1 Exposure |       | Fog |
|-----------|-----------------|----------------|-------|----------------|-------|-----|
|           |                 | Speed          | Gamma | Speed          | Gamma |     |
| Control   |                 | 540            | 1.81  | 430            | 1.87  | .56 |
| I         |                 | 620            | 2.27  | 430            | 2.02  | .74 |
| I plus II |                 | 750            | 2.06  | 470            | 2.26  | .33 |

## ONE WEEK AT 120° F. AND 65% R.H.

| Compound  |  | Fog  |
|-----------|--|------|
| Control   |  | .48  |
| I         |  | 1.18 |
| I plus II |  | .38  |

## Example 12

A gelatino-silver iodobromide emulsion, digested with sulfur and gold compounds was divided into three portions. One portion was treated with 0.5 g. of the polyoxyethylated oleyl alcohol of Example 1 per mole of silver halide. To a second portion was added 0.5 g. ("Emulphor ON") per mole of silver halide together with 10 millimoles of p-t-amyphenol (II).

Coating, exposure, development and aging were carried out as in Example 4.

## FRESH RESULTS

| Compound                          | Amount per Mole         | No. 2 Exposure |       | No. 1 Exposure |       | Fog |
|-----------------------------------|-------------------------|----------------|-------|----------------|-------|-----|
|                                   |                         | Speed          | Gamma | Speed          | Gamma |     |
| Control                           | None                    | 720            | 2.27  | 400            | 2.01  | .38 |
| I Polyoxyethylated oleyl alcohol. | .5 g.                   |                |       |                |       | .72 |
| I plus II                         | .5 g.<br>10 millimoles. | 950            | 2.73  | 610            | 2.19  | .40 |

10  
ONE MONTH ROOM AGING

| Compound  | No. 2 Exposure |       | No. 1 Exposure |       | Fog |
|-----------|----------------|-------|----------------|-------|-----|
|           | Speed          | Gamma | Speed          | Gamma |     |
| Control   |                |       |                |       | .56 |
| I plus II | 800            | 2.47  | 490            | 2.11  | .36 |

10  
ONE WEEK AT 120° F. AND 65% R.H.

| Compound  |  | Fog |
|-----------|--|-----|
| Control   |  | .48 |
| I plus II |  | .52 |

## Example 13

A gelatino-silver iodobromide emulsion, digested with sulfur and gold compounds, was divided into three portions. One portion was treated with 1.1 g. of the condensation product of Example 1 per mole of silver halide. To a second portion was added 1.1 g. of the condensation product per mole of silver halide together with 20 millimoles of 2,4-di-sec-amylphenol (II).

Coating, exposure, development and aging were carried out as in Example 4.

## FRESH RESULTS

| Compound                          | Amount per Mole          | No. 2 Exposure |       | No. 1 Exposure |       | Fog |
|-----------------------------------|--------------------------|----------------|-------|----------------|-------|-----|
|                                   |                          | Speed          | Gamma | Speed          | Gamma |     |
| Control                           | None                     | 690            | 2.54  | 480            | 2.19  | .37 |
| I Polyoxyethylated oleyl alcohol. | 1.1 g.                   |                |       |                |       | .48 |
| I plus II                         | 1.1 g.<br>20 millimoles. | 760            | 3.17  | 490            | 2.49  | .32 |

## ONE MONTH ROOM AGING

| Compound  | Amount per Mole | No. 2 Exposure |       | No. 1 Exposure |       | Fog |
|-----------|-----------------|----------------|-------|----------------|-------|-----|
|           |                 | Speed          | Gamma | Speed          | Gamma |     |
| Control   |                 | 670            | 2.25  | 400            | 1.93  | .28 |
| I         |                 | 850            | 2.58  | 400            | 2.05  | .36 |
| I plus II |                 | 690            | 3.03  | 400            | 2.39  | .21 |

55  
ONE WEEK AT 120° F. AND 65% R.H.

| Compound  |  | Fog |
|-----------|--|-----|
| Control   |  | .57 |
| I         |  | .90 |
| I plus II |  | .31 |

60  
Example 14

A gelatino-silver iodobromide emulsion, digested with sulfur and gold compounds, was divided into three portions. One portion was treated with 0.5 g. of the condensation product of Example 1 per mole of silver halide. To a second portion was added 0.5 g. of the above condensation product per mole of silver halide together with 20 millimoles of p-n-butylphenol (II).

Coating, exposure, development and aging were carried out as in Example 4.

## FRESH RESULTS

| Compound                            | Amount per Mole          | No. 2 Exposure |       | No. 1 Exposure |       | Fog |
|-------------------------------------|--------------------------|----------------|-------|----------------|-------|-----|
|                                     |                          | Speed          | Gamma | Speed          | Gamma |     |
| Control                             | None                     | 720            | 2.40  | 420            | 2.13  | .25 |
| Polyoxyethylated oleyl alcohol (I). | 0.5 g.                   |                |       |                |       | .50 |
| I plus II                           | 0.5 g.<br>20 millimoles. | 960            | 2.55  | 430            | 2.22  | .26 |

## ONE MONTH ROOM AGING

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 690            | 2.18  | 350            | 1.83  | .20 |
| I plus II | 0.5 g.<br>20 millimoles. | 940            | 2.58  | 430            | 2.06  | .15 |

## Example 15

A gelatino-silver iodobromide emulsion, digested with sulfur and gold compounds, was divided into three portions. One portion was treated with 0.5 g. of the condensation product of Example 1 per mole of silver halide. To a second portion was added 0.5 g. of the above condensation product per mole of silver halide together with 20 millimoles of p-isobutylphenol (II).

Coating, exposure, development and aging were carried out as in Example 1.

## FRESH RESULTS

| Compound                            | Amount per Mole          | No. 2 Exposure |       | No. 1 Exposure |       | Fog |
|-------------------------------------|--------------------------|----------------|-------|----------------|-------|-----|
|                                     |                          | Speed          | Gamma | Speed          | Gamma |     |
| Control                             | None                     | 720            | 2.40  | 420            | 2.13  | .25 |
| Polyoxyethylated oleyl alcohol (I). | 0.5 g.                   |                |       |                |       | .50 |
| I plus II                           | 0.5 g.<br>20 millimoles. | 970            | 2.71  | 440            | 2.23  | .26 |

## ONE MONTH ROOM AGING

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 690            | 2.18  | 350            | 1.83  | .20 |
| I plus II | 0.5 g.<br>20 millimoles. | 880            | 2.50  | 420            | 2.11  | .22 |

## ONE WEEK AT 120° F. AND 65% R.H.

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 690            | 2.18  | 350            | 1.83  | .20 |
| I         | 0.5 g.                   |                |       |                |       | .44 |
| I plus II | 0.5 g.<br>20 millimoles. | 880            | 2.50  | 420            | 2.11  | .22 |

## Example 16

A gelatino-silver iodobromide emulsion, digested with sulfur and gold compounds, was divided into three portions. One portion was treated with 0.5 g. of the condensation product of Example 1 per mole of silver halide. To a second portion there was added 0.5 g. of the above condensation product together with 20 millimoles of 2,6-di-t-butyl-4-methylphenol (II). Neither of these additions was made to a third portion.

Coating, exposure, development and aging were carried out as in Example 1.

## FRESH RESULTS

| Compound                            | Amount per Mole          | No. 2 Exposure |       | No. 1 Exposure |       | Fog  |
|-------------------------------------|--------------------------|----------------|-------|----------------|-------|------|
|                                     |                          | Speed          | Gamma | Speed          | Gamma |      |
| Control                             | None                     | 690            | 2.66  | 410            | 2.34  | 0.10 |
| Polyoxyethylated oleyl alcohol (I). | 0.5 g.                   | 850            | 2.88  | 430            | 2.15  | 0.35 |
| I plus II                           | 0.5 g.<br>20 millimoles. | 760            | 2.76  | 420            | 2.19  | 0.26 |

## ONE WEEK AT 120° F. AND 65% R.H.

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 690            | 2.69  | 300            | 2.20  | .22 |
| I         | 0.5 g.                   |                |       |                |       | .48 |
| I plus II | 0.5 g.<br>20 millimoles. | 660            | 3.46  | 330            | 2.40  | .26 |

## Example 17

A gelatino-silver iodobromide emulsion, digested with sulfur and gold compounds, was divided into three portions. One portion was treated with 0.5 g. of the polyethylene oxide (I) compound described in Example 3 per mole of silver halide. To a second portion was added 0.5 g. of the polyethylene oxide compound together with 20 millimoles of 2,4-di-t-amylphenol (II). Neither of these additions was made to a third portion.

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 690            | 2.69  | 300            | 2.20  | .22 |
| I         | 0.5 g.                   |                |       |                |       | .48 |
| I plus II | 0.5 g.<br>20 millimoles. | 660            | 3.46  | 330            | 2.40  | .26 |

## ONE MONTH ROOM AGING

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 640            | 2.29  | 330            | 1.83  | .22 |
| I         | 0.5 g.                   |                |       |                |       | .63 |
| I plus II | 0.5 g.<br>20 millimoles. | 610            | 3.49  | 290            | 2.37  | .24 |

## ONE WEEK AT 120° F. AND 65% R.H.

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     | 640            | 2.29  | 330            | 1.83  | .22 |
| I         | 0.5 g.                   |                |       |                |       | .63 |
| I plus II | 0.5 g.<br>20 millimoles. | 610            | 3.49  | 290            | 2.37  | .24 |

## Example 18

A gelatino-silver iodobromide emulsion, digested with sulfur and gold compounds, was divided into three portions. One portion was treated with 0.5 g. of the polyethylene oxide of Example 3 (I) per mole of silver halide. To a second portion was added 0.5 g. of (I) together with 20 millimoles of p-alpha-cumylphenol (II). Neither of these additions was made to a third portion.

Coating, exposure, processing and aging were carried out as in Example 1.

## FRESH RESULTS

| Compound | Amount per Mole     | No. 2 Exposure |       | No. 1 Exposure |       | Fog |
|----------|---------------------|----------------|-------|----------------|-------|-----|
|          |                     | Speed          | Gamma | Speed          | Gamma |     |
| Control  | None                | 860            | 2.70  | 380            | 2.34  | .15 |
| I        | 0.5 g.              | 1,010          | 2.35  | 490            | 1.91  | .36 |
| I plus   | 0.5 g.              |                |       |                |       |     |
| II       | 20 milli-<br>moles. | 810            | 2.71  | 400            | 2.46  | .14 |

## ONE MONTH ROOM AGING

| Compound  | No. 2 Exposure |       | No. 1 Exposure |       | Fog |
|-----------|----------------|-------|----------------|-------|-----|
|           | Speed          | Gamma | Speed          | Gamma |     |
| Control   | 700            | 2.19  | 320            | 2.11  | .13 |
| I         |                |       |                |       | .70 |
| I plus II | 720            | 2.53  | 330            | 2.49  | .12 |

## ONE WEEK AT 120° F. AND 65% R.H.

| Compound | Fog  |
|----------|------|
| Control  | .22  |
| I        | 1.98 |
| I and II | .18  |

## Example 19

A gelatino-silver iodobromide emulsion containing 6.8 mole percent iodide and optically sensitized with a mixture of two carbocyanine dyes was divided into three portions. One portion was treated with 0.3 g., per mole of silver halide, of a polyethylene oxide (I) having an average molecular weight of 3000-3700 ("Carbowax 4000" made by Carbide and Carbon Chemicals Company). To a second portion there was added 0.3 g. of the polyethylene oxide compound together with 5.3 g. of the mixture (II) of phenols described in Example 9. To a third portion there was added 0.3 g. of (I) per mole of silver halide and 10.6 g. of (II).

The emulsion was coated, dried and exposed to a white light and to a red light and processed in the conventional manner. Speed is given in terms of a reciprocal of exposure at a density of 0.2.

## FRESH RESULTS

| Compound | Amount per Mole | White Light |       | Fog | Red Filter Factor |
|----------|-----------------|-------------|-------|-----|-------------------|
|          |                 | Speed       | Gamma |     |                   |
| I        | 0.3             | 480         | 1.06  | .12 | 4.0               |
| I plus   | 0.3             |             |       |     |                   |
| II       | 5.3             | 460         | 1.00  | .11 | 3.5               |
| I plus   | 0.3             |             |       |     |                   |
| II       | 10.6            | 480         | .91   | .09 | 3.7               |

## ONE WEEK AT 120° F. AND 65% R.H.

| Compound | Amount | Fog |
|----------|--------|-----|
|          | g.     |     |
| I        | 0.3    | .09 |
| I plus   | 0.3    |     |
| II       | 5.3    | .08 |
| I plus   | 0.3    |     |
| II       | 10.6   | .08 |

## Example 20

A gelatino-silver iodobromide emulsion, digested with sulfur and gold compounds, was divided into three portions. One portion was treated with 0.5 g. per mole of silver halide of the condensation product described in Example 1 ("Emulphor" ON) (I). To a second portion was added 0.5 g. of (I) together with 20 millimoles of 2-sec-butyl-4-ethylphenol (II). Neither of these additions was made to a third portion.

Coating, exposure, processing and aging were carried out as in Example 1.

## FRESH RESULTS

| 5       | Compound            | Amount per Mole | No. 2 Exposure |       | No. 1 Exposure |       | Fog |
|---------|---------------------|-----------------|----------------|-------|----------------|-------|-----|
|         |                     |                 | Speed          | Gamma | Speed          | Gamma |     |
| Control | None                |                 |                |       |                |       | .45 |
| I       | 0.5 g.              |                 |                |       |                |       | .58 |
| I plus  | 0.5 g.              |                 |                |       |                |       |     |
| II      | 20 milli-<br>moles. |                 |                |       |                |       |     |

## 10 TWO MONTHS AGING

| 15        | Compound | No. 2 Exposure |       | No. 1 Exposure |       | Fog |
|-----------|----------|----------------|-------|----------------|-------|-----|
|           |          | Speed          | Gamma | Speed          | Gamma |     |
| Control   | None     |                |       |                |       | .46 |
| I plus II | 780      | 2.81           | 420   | 2.35           | .40   |     |

The 2-sec-butyl-4-ethylphenol was prepared by the Clemmenson reduction of 2-sec-butyl-4-hydroxyacetophenone. The latter ketone was prepared by the Friedel-Crafts acylation of o-sec-butylphenol with acetyl chloride in the presence of aluminum chloride by the general procedure of Rosenmund and Schulz. Arch. Pharmaz. deut. pharm. Ges., 265, 308 (1927). The ketone was reduced by the general method of Clemmenson [Ber. 47, 53 (1914)] and a portion of the resulting product was redistilled to give a colorless liquid having a boiling point of 136-138°/18 mm.

35. *Example 21*  
2-ethyl-4-isopropylphenol was prepared by the Clemmenson reduction of 2-acetyl-4-isopropylphenol by the procedure described in Ber. 47, 53 (1914). The ketone was prepared by the acylation of p-isopropylphenol with acetyl chloride in the presence of  $\text{AlCl}_3$  by the general procedure of Sandulesco & Gerard, Bull. Soc. Chim. [4] 47, 1300 (1930).

45. A gelatino-silver iodobromide emulsion, digested with sulfur and gold compounds, was divided into three portions. One portion was treated with 0.5 g., per mole of silver halide, of the condensation product described in Example 1 (I). To a second portion there was added 0.5 g. of (I) together with 20 millimoles of 2-ethyl-4-isopropylphenol (II). Neither of these additions was made to a third portion.

50. Coating, exposure, processing and aging was carried out as described in Example 1.

| 55      | Compound            | Amount per Mole | No. 2 Exposure |       | No. 1 Exposure |       | Fog |
|---------|---------------------|-----------------|----------------|-------|----------------|-------|-----|
|         |                     |                 | Speed          | Gamma | Speed          | Gamma |     |
| Control | None                |                 |                |       |                |       | .45 |
| I       | 0.5 g.              |                 |                |       |                |       | .58 |
| I plus  | 0.5 g.              |                 |                |       |                |       |     |
| II      | 20 milli-<br>moles. |                 |                |       |                |       |     |

## 60 TWO MONTHS AGING

| 70      | Compound            | Amount per Mole | No. 2 Exposure |       | No. 1 Exposure |       | Fog |
|---------|---------------------|-----------------|----------------|-------|----------------|-------|-----|
|         |                     |                 | Speed          | Gamma | Speed          | Gamma |     |
| Control | None                |                 |                |       |                |       | .46 |
| I       | 0.5 g.              |                 |                |       |                |       | .38 |
| I plus  | 0.5 g.              |                 |                |       |                |       |     |
| II      | 20 milli-<br>moles. |                 |                |       |                |       |     |

## 75 TWO MONTHS AGING

## Example 22

A gelatino-silver iodobromide emulsion, digested with sulfur and gold sensitizing compounds, was divided into three portions. One portion was treated with 0.5 g., per mole of silver halide, of the polyethylene oxide compound (I) of Example 1. To a second portion there was added 0.5 g. of (I) and 20 millimoles of a 2-methyl-4-ethylphenol (II) per mole of silver halide. Neither of these additions was added to a third portion.

Coating, exposure, processing and aging were carried out as in Example 1.

## FRESH RESULTS

| Compound  | Amount per Mole          | No. 2 Exposure |       | No. 1 Exposure |       | Fog |
|-----------|--------------------------|----------------|-------|----------------|-------|-----|
|           |                          | Speed          | Gamma | Speed          | Gamma |     |
| Control   | None                     |                |       |                |       | .45 |
| I         | 0.5 g.                   |                |       |                |       | .58 |
| I plus II | 0.5 g.<br>20 millimoles. | 850            | 3.67  | 400            | 2.99  | .38 |

## TWO MONTHS AGING

| Compound  | Amount per Mole | No. 2 Exposure |       | No. 1 Exposure |       | Fog |
|-----------|-----------------|----------------|-------|----------------|-------|-----|
|           |                 | Speed          | Gamma | Speed          | Gamma |     |
| Control   | None            |                |       |                |       | .46 |
| I         | 740             | 3.29           | 330   | 2.49           | .38   |     |
| I plus II | 760             | 3.41           | 360   | 2.76           | .23   |     |

## Example 23

A gelatino-silver iodobromide emulsion, digested with sulfur and gold sensitizers, was divided into three portions. One portion was treated with 0.67 g. of the polyethylene oxide-oleyl alcohol condensation product (I) of Example 1 per mole of silver halide. To a second portion there was added 0.67 g. of (I) and 10 millimoles of 2-n-octyl-4,5-dimethylphenol (II) per mole of silver halide. Neither of these additions was made to a third portion which served as a control. Coating, exposure and development were carried out as in Example 1 with the following results:

## FRESH RESULTS

| Compound  | Amount per Mole           | No. 2 Exposure |       | No. 1 Exposure |       | Fog |
|-----------|---------------------------|----------------|-------|----------------|-------|-----|
|           |                           | Speed          | Gamma | Speed          | Gamma |     |
| Control   | None                      |                |       |                |       | .27 |
| I         | 0.67 g.                   | 880            | 2.39  | 430            | 2.01  | .59 |
| I plus II | 0.67 g.<br>10 millimoles. | 1,030          | 2.60  | 455            | 2.30  | .36 |

## ONE MONTH ROOM AGING

| Compound  | Amount per Mole | No. 2 Exposure |       | Fog |
|-----------|-----------------|----------------|-------|-----|
|           |                 | Speed          | Gamma |     |
| Control   | None            | 810            | 2.19  | .37 |
| I plus II | 1,025           |                | 2.78  | .30 |

## ONE WEEK AT 120° F. AND 65% R.H.

| Compound  | Fog  |
|-----------|------|
| Control   | .48  |
| I         | 1.60 |
| I plus II | .66  |

The 2-n-octyl-4,5-dimethylphenol (B.P.138° C./1 mm.;  $(n)_D^{25}$  1.5060) was prepared by the Clemmensen reduction of 2-n-octanoyl-4,5-dimethylphenol. The ketone

## 16

was obtained from the Friedel-Crafts acylation of 3,4-dimethylphenol with n-octanoyl chloride in the presence of aluminum chloride.

In place of the specific hydrocarbon-substituted mononuclear monohydric phenols used in the foregoing examples there may be substituted one or more other such compounds falling within the generic characterization given above. Suitable additional compounds include 4-t-butyl-3-methylphenol, 2- $\alpha$ -methyl-benzyl-4-t-butylphenol, p-phenylphenol, p-sec.-butylphenol, and 2-t-butyl-4-methylphenol. These compounds are generally added after digestion and after addition of the polyoxyalkylene sensitizing compound. At the same time other compounds having antifogging properties can be added to the emulsions. Suitable antifogging agents which can be used include benzotriazole, nitrobenzimidazole, 1-phenyl-5-mercaptopetetrazole, and benzothiazole.

The resulting photographic emulsions can be coated onto any suitable support to make the desired type of photographic element. Suitable supports include cellulose esters, e.g., cellulose acetate, cellulose nitrate, cellulose acetate butyrate, cellulose propionate; super polymers, e.g., nylon, polyethylene terephthalate, polyvinyl chloride, vinylidene chloride copolymers with vinyl acetate, acrylonitrile, etc.; metal sheets or foils, e.g., aluminum and zinc; and paper including resin-coated and baryta-coated paper; as well as glass plates, *inter alia*.

An advantage of the invention is that it provides photographic emulsions and elements with improved stability and aging characteristics. It enables one to obtain the useful sensitizing action of the polyoxyalkylene compounds without an undue degree of fog being formed upon storage of the photographic elements for long periods.

Another advantage is that the improved emulsions and emulsion layers can be made by the addition of readily available chemical compounds. A further advantage is that the improved emulsions do not require the use of expensive chemicals or tedious procedures. A still further advantage is that the speed of the aforescribed silver halide emulsions to light of various intensities is not affected to the same degree as known non-phenolic antifogging agents. A related advantage is that while the hydrocarbon-substituted mononuclear monohydric phenols have an antifogging action in photographic silver halide emulsions sensitized with polyoxyalkylene compounds, they do not have a significant effect on other photographic properties, e.g., contrast, graininess, resolution, optical sensitization and latent image stability.

I claim:

1. A photographic, water-permeable colloid-silver halide emulsion containing per mole of silver halide (1) from 0.1 to 2.0 grams of a non-optical sensitizing agent having a molecular weight of at least 282 and containing at least 2 oxyalkylene units of 2 to 4 carbon atoms and being taken from the group consisting of polyalkylene ether glycols, and condensation products of alkylene oxides of 2 to 4 carbon atoms with monohydric alcohols, glycols, fatty acids, saturated aliphatic amines, and hexitol ring dehydration products, and (2) from 5 to 50 millimoles of at least one hydrocarbon-substituted monohydric phenol of at least 9 carbon atoms having a hydrocarbon substituent in the para-position to the hydroxyl group and 0 to 4 additional hydrocarbon substituents in the remainder of the benzene ring, said hydrocarbon substituents being the sole substituents in said phenol and being taken from the group consisting of alkyl, aryl, aralkyl and cycloalkyl substituents.

2. An emulsion as set forth in claim 1 wherein at least one of the said hydrocarbon substituents is a butyl substituent.

3. An emulsion as set forth in claim 1 wherein the hydrocarbon substituent in the para-position is an alkyl radical of 1 to 12 carbon atoms.

4. An emulsion as set forth in claim 1 wherein said

monohydric phenol is 2-benzyl-4-methyl-6-t-butylphenol.  
 5. An emulsion as set forth in claim 1 wherein said sensitizing agent is the condensation product of ethylene oxide with oleyl alcohol having a molecular weight of at least 300.

6. An emulsion as set forth in claim 1 wherein said sensitizing agent is a polyethylene ether glycol having an average molecular weight of at least 1500.

7. An emulsion as set forth in claim 1 wherein said silver halide is iodobromide.

8. An element as set forth in claim 1 wherein said colloid is gelatin.

9. A photographic element comprising a support bearing at least one layer composed of an emulsion as set forth in claim 1.

5

10. An element as set forth in claim 9 wherein said support is a hydrophobic film base.

11. An element as set forth in claim 9 wherein said support embodies a polyethylene terephthalate film base.

15

References Cited in the file of this patent

## UNITED STATES PATENTS

|           |                 |               |
|-----------|-----------------|---------------|
| 2,341,877 | Middleton       | Feb. 15, 1944 |
| 2,441,389 | Blake           | May 11, 1948  |
| 2,594,917 | Gunther         | Apr. 29, 1952 |
| 2,596,742 | Vaughn et al.   | May 13, 1952  |
| 2,752,246 | Weaver          | June 26, 1956 |
| 2,756,147 | Reynolds et al. | July 24, 1956 |